

## UNITED STATES PATENT OFFICE

WILLIAM THEODORE ANDERSON, JR., AND LESTER FLETCHER BIRD, OF NEWARK, NEW JERSEY, ASSIGNEES TO HANOVIA CHEMICAL AND MANUFACTURING COMPANY, OF NEWARK, NEW JERSEY, A CORPORATION OF NEW JERSEY

## METHOD OF FORMING COPPER COPPER-OXIDE RECTIFIER PLATES

No Drawing.

Application filed August 30, 1928. Serial No. 303,122.

Copper-copper oxide rectifier plates have been prepared in various ways. Ordinarily the method followed consisted in heating a prepared copper plate to a high temperature in an oxidizing atmosphere, and producing a layer of red oxide on the whole surface, cooling the plate somewhat in an oxidizing atmosphere during which the surface of the red oxide is further oxidized causing the formation of black oxide and then reducing in a reducing solution or liquid.

The action of the reducing agent was two-fold. The black oxide formed by the oxidation of the red oxide during the cooling process was reduced to copper and more or less of the surface of the red oxide was also reduced to copper. The copper formed was peculiar in that its molecular structure varied with the conditions under which it was produced. As the structure could not be seen its exact character was not visually ascertainable but as soon as the rectifier plate was inserted in an electric circuit the structure of the formed copper became apparent because of the resistance of the contact between it and the oxide.

Copper-copper oxide junctions exhibit very peculiar properties that are not understood because the molecular structure of the contact determines its electrical characteristics. Under certain conditions of formation such a junction will act as a very good rectifier of electric currents and under other conditions of formation no rectification will occur and the contact will behave like any ordinary bilateral contact. The determining condition seems to be the concentration of the active reducing material at the surface of the copper oxide. It seems that junctions formed in the presence of concentrated reducing agents, like pure vapors, are rectifiers, and junctions formed in the presence of sufficiently dilute agents are non-rectifiers.

Since the object of the reducing agent is to produce copper on the outside of the oxide which does not form a rectifying contact with the copper oxide, it must be formed under conditions that are capable of control as to concentration of the active material and without coming in contact with any pure ac-

tive vapors. It will be immediately recognized that this condition is difficult to secure. The copper oxide must be reduced at a fairly high temperature in order for the process to be successful. However, if an active gas is formed by the reducing process and is present when the black oxide is reduced, the concentration of reducing agent in the vapor is too high and the formed copper will not be arranged in the proper molecular structure so that the efficiency of the plate will be seriously reduced.

The problem simplified to its component parts involves the use of an active reducing agent that is non-volatile at a temperature approaching 500° C. By far the larger number of organic acids, aldehydes, alcohols etc. which any skilled chemist recognizes as reducing agents for hot copper oxide are very volatile at 500° C. and obviously any solution of these in water will volatilize a few degrees above 100° C.

Aqueous solutions of many of them will work with varying degrees of success especially a solution of wood alcohol in water but this solution was found to be critical to the temperature of the plate when reduced and also critical to the strength of the solution of alcohol. Moreover, it was found that the oxide on the copper plates was strained severely by the sudden cooling from 500° C. or thereabouts to the temperature of the water and alcohol at about 20° C. In many cases the oxide was cracked and broken free from the copper. The rectifying contact is only secured by having the oxide adhere rigidly to the copper and any broken or loose crystals of the oxide that might be present against the copper at the junction produce serious leakage of the plates for current in the reverse direction and materially reduce the effectiveness of the rectification.

Paraffine oil was found to be fairly non-volatile at about 500° C. but was so inactive that it would not reduce the copper oxide at this temperature. Successful reduction occurred at a somewhat higher temperature but not below the volatilization point and the copper so formed was in the wrong molecular arrangement.

The answer apparently depended upon an activating agent that could be placed in the paraffine so that the paraffine would be saturated with the vapor of the active material and the necessary reduction takes place below the temperature at which the paraffine would react but still without any active vapor being formed. Several substances were found that would work in such a combination. Among these was hydrochinon. The solution of hydrochinon and paraffine could be heated so that the vapor pressure of the hydrochinon in the paraffine was appreciable and the activity of the solution was controlled by the temperature. The vapor pressure of the hydrochinon was of course equal to atmospheric pressure at 169° C. so that this was the limiting temperatures of the solution. The paraffine becomes a liquid at about 70° C. so that the range of possible operation lay between 70° C. and 169° C.

It is well known that when two liquids that are normally immiscible are in contact each diffuses somewhat into the other so that a vapor pressure of each is present in the other. For this reason oil and water in contact mix to a certain extent, air and water mix so that the water is saturated with air and the air with water vapor. Very few substances are soluble in paraffine and at ordinary temperatures it is very inert chemically. However, when paraffine is melted and in contact with many liquid substances, with which no chemical reaction occurs, the vapor of the foreign substance penetrates the paraffine and exists in concentrations in it depending upon the temperature and pressure of the mixture.

When an excess of the foreign liquid is in contact with it the paraffine is in a state of saturated equilibrium with the foreign liquid vapor. This characteristic of vapor diffusion provides an almost ideal condition for a suitable reducing agent, in the treatment of the rectifier plates, because an active agent can be added to the paraffine and only the vapor of this agent exists in a very low concentration in the paraffine, moreover this concentration is controllable by variation of the operating temperature. Certain of the alcohols, aldehydes, ketones, organic acids, and hydrocarbons possess the necessary characteristics for satisfactory operation as an activating agent for a paraffine reducing solution. These characteristics may be listed as follows:

1. The specific gravity at 150° to 200° C. must be above that of melted paraffine at these temperatures so the active material remains at the bottom of the containing vessel. Otherwise the prepared copper plates would have to pass thru the active material to enter the paraffine and so would be destroyed.

2. The substance must be an active reducing agent so that copper oxides of both types

are readily attacked at temperatures between 200° and 500° C.

3. The boiling point of the substance should be about 150° C. or higher depending upon its activity as a reducing agent.

4. The unwanted products of the reaction between the active substance and the oxide should be gaseous at the temperature of the solution and so boil off. When possible the reaction products should not be poisonous.

The use of the reducing methods described offers several distinct advantages as evidenced by the following summary.

First: The nature of the contact between the reduced copper and the oxide is very vital and must be controlled so that the most efficient bilateral contact is secured. The reducing materials and the methods described make such control possible and exact.

Second: The activity of the reducing material is ordinarily dependent upon the temperature at which the oxidized rectifier plates are immersed. It has been shown that this may not be a satisfactory method since the temperature required for proper activity may be above that allowable to secure proper molecular structure of the formed copper. The reducing materials described present special advantages for this purpose since the activity of the reducing agent can be varied within itself and is not dependent upon a high temperature of the oxidized plate when immersed.

Third: This reducing medium permits the use of an active volatile material for the reducing agent without having the active gas of this material operating as an uncontrollable reducing agent. Only a limited concentration of the active vapor can be active on any plate at any instant.

Fourth: The reducing medium described offers another distinct advantage in that the plates come out being sealed automatically against moisture with a complete paraffine coating. Sufficient paraffine normally adheres to the plate so that it is sealed. This feature contributes somewhat toward ease of handling of the plates.

We claim:

1. A bath for reducing copper oxide, comprising paraffine and hydrochinon, the paraffine serving as an inert vehicle to hold and distribute the hydrochinon.

2. A bath for reducing copper oxide, comprising paraffine and a vapor of a hydrocarbon reducing substance, the paraffine serving as an inert vehicle to hold and distribute the reducing substance.

3. In the manufacture of copper-copper oxide rectifier plates, a bath for reducing copper oxide to provide a film of metallic copper, said bath comprising hydrochinon and a substance inactive with copper oxide to serve as a vehicle to hold and distribute the hydrochinon.

4. In the manufacture of copper-copper oxide rectifier plates, the method of reducing copper oxide consisting of quenching in a bath of paraffine and hydrochinon.

5. A bath for reducing copper oxide, comprising paraffin, and a vapor of a hydrocarbon derivative reducing substance, the paraffin serving as an inert vehicle to hold and distribute the reducing substance.

10 This specification signed this 17th day of August, 1928.

WILLIAM THEODORE ANDERSON, Jr.  
LESTER FLETCHER BIRD.

15

20

25

30

35

40

45

50

55

60